

1

3,429,772

## MANUFACTURE OF PAPER

Roland Michael Harvey, Leicester, and Christopher Richard Napier Johnson, Braintree, England, assignors to Chemstrand Limited, London, England

No Drawing. Filed June 1, 1965, Ser. No. 460,534  
Claims priority, application Great Britain, June 3, 1964,  
23,014/64

U.S. Cl. 162—157  
Int. Cl. D21h 5/20

9 Claims

## ABSTRACT OF THE DISCLOSURE

By treatment with oxygen-forming agents, fibres formed from acrylonitrile polymers containing at least 80 percent by weight acrylonitrile split into sub-deniers requiring less beating than untreated fibres and when formed into paper sheets by conventional papermaking methods exhibit enhanced physical properties as tear and bursting strengths. Preferable oxygen-forming agents are potassium permanganate or ammonium persulphate.

This invention relates to the manufacture of paper formed from acrylonitrile polymer fibres. It is an object of the invention to increase the ease with which such fibres can be beaten, to provide a paper-making stock, in a conventional beater, refiner or stockmaker and to enable a paper to be produced having improved physical properties.

According to one aspect of the present invention there is provided a process for the treatment of fibres formed of an acrylonitrile polymer containing at least 80 percent by weight of acrylonitrile to render said fibres suitable for use in the manufacture of paper, comprising the steps of reducing said fibres to staple lengths, immersing said fibres in an aqueous solution of an oxygen-forming agent at a temperature in the range of from 10° C. to 100° C. for a predetermined period, thereby to partially disrupt said fibres, washing said fibres to remove said oxygen-forming agent and drying said fibres. The invention also includes fibres when treated by such process.

According to another aspect of the invention there is provided a process for the manufacture of paper from fibres produced from an acrylonitrile polymer containing at least 80 percent by weight of acrylonitrile, comprising the steps of reducing said fibres to staple lengths, immersing said fibres in an aqueous solution of an oxygen-forming agent at a temperature in the range of from 10° C. to 100° C. for a predetermined period, thereby to partially disrupt said fibres, washing said fibres to remove said oxygen-forming agent, drying said fibres, beating said fibres in an aqueous dispersion and forming said fibres into a paper sheet or web. The invention also includes paper when produced by such process.

Preferably the oxygen-forming agents employed in carrying out the invention are potassium permanganate, or ammonium persulphate. Other agents which may be employed are sodium hypochlorite, sodium perborate, potassium bichromate and potassium persulphate. Other oxygen-forming agents that may be found suitable can be employed, including mixtures of any of the said agents.

It has been found that fibres which have been subjected to treatment in an aqueous solution of an oxygen-forming agent in accordance with the invention are partially disrupted and, when subjected to beating, are split into sub-deniers therefore require a lesser amount of beating than fibres which have not been treated in the manner referred to. When the fibres treated in accordance with the invention are formed into paper webs or sheets by conventional paper-making methods they exhibit enhanced physical properties, notably as regards tear and bursting strengths.

2

The fibres treated by the invention can be prepared from polyacrylonitrile, copolymers, including binary and ternary polymers containing at least 80 percent by weight of acrylonitrile in the polymer molecule or a blend comprising polyacrylonitrile or copolymers comprising acrylonitrile with 2 to 50 percent by weight of the blend of another polymeric material, the blend having an overall polymerized acrylonitrile content of at least 80 percent by weight. For example, the polymer from which the fibres are prepared may be a copolymer of from 80 to 98 percent by weight of acrylonitrile and from 2 to 20 percent by weight of another monomer containing  $>C=C<$  linkage and copolymerizable with acrylonitrile. Suitable copolymerizable mono-olefinic monomers include acrylic, alpha-chloroacrylic and methacrylic acids, the methacrylates, such as methyl methacrylate, ethyl methacrylate, butyl methacrylate, methoxymethyl methacrylate, beta-chloroethyl methacrylate, and the corresponding esters of acrylic and alpha-chloroacrylic acids; vinyl chloride, vinyl fluoride, vinyl bromide, vinylidene chloride, 1-chloro-1-bromoethylene; methacrylonitrile; acrylamide and methacrylamide; alpha-chloroacrylamide, or monoalkyl substitution products thereof; methyl vinyl ketone; vinyl carboxylates, such as vinyl acetate, vinyl chloroacetate, vinyl propionate, and vinyl stearate; N-vinylimides, such as N-vinylphthalimide and N-vinylsuccinimide; methylene malonic esters; itaconic acid and itaconic esters; N-vinylcarbazole; vinyl furane; alkyl vinyl ethers; vinyl sulphonic acid; ethylene alpha, beta-dicarboxylic acids or their anhydrides or derivatives, such as diethyl citraconate and diethyl mesaconate, styrene, vinyl naphthalene, vinyl-substituted tertiary teterocyclic amines, such as the vinylpyridines and alkyl-substituted vinylpyridines, for example, 2-vinylpyridine, 4-vinylpyridine and 2-methyl-5-vinylpyridine; 1-vinylimidazole and alkyl substituted 1-vinylimidazoles, such as 2,4,5-methyl-1-vinylimidazole, vinyl pyrrolidone or vinyl piperidone.

The polymer can be a ternary polymer or higher interpolymer, for example products obtained from the interpolymerization of acrylonitrile and two or more of any of the monomers, other than acrylonitrile enumerated above. More specifically, and preferably the ternary polymer comprises acrylonitrile, methacrylonitrile and 2-vinylpyridine. The ternary polymers preferably contain from 80 to 98 percent by weight of acrylonitrile, from 1 to 10 percent by weight of a vinylpyridine or a 1-vinylimidazole, and from 1 to 18 percent by weight of another copolymerizable mono-olefinic substance, such as methacrylonitrile or vinyl chloride.

The polymer can also be a blend of a polyacrylonitrile or of a binary interpolymer of from 80 to 98 percent by weight of acrylonitrile and from 1 to 20 percent by weight of at least one other  $>C=C<$  containing substance with from 2 to 50 percent of the weight of the blend of a copolymer of from 10 to 70 percent by weight of acrylonitrile and from 30 to 90 percent by weight of at least one other  $>C=C<$  containing polymerizable monomer. Preferably, when the polymeric material comprises a blend it will be a blend of a terpolymer of 90 to 98 percent by weight of acrylonitrile and from 2 to 10 percent by weight of another mono-olefinic monomer, such as a vinyl acetate, which is not receptive to dyestuff, with a sufficient amount of a copolymer of from 10 to 70 percent by weight of acrylonitrile and from 30 to 90 percent by weight of a vinyl-substituted tertiary heterocyclic amine, such as a vinylpyridine or 1-vinylimidazole, to give a dyeable blend having an overall vinyl-substituted tertiary heterocyclic amine content of from 2 to 10 percent, based on the weight of the blend.

For a better understanding of the invention the following examples are given in which all percentages are by weight unless otherwise stated.

## Example I

In this example 100 grams dry weight undried acrylonitrile polymer fibers of 3 denier sold under the registered trademark Acrilan 1656 were cut into 1 inch staple lengths and added to 5.9 litres of water contained in the trough of a Clough laboratory beater. A counter-weight of 3 1/4 lbs. was placed on the lever arm of the beater and the clearance between the roll and bedplate was set at 7 mil. Beating was carried out at 1000 ft./min. peripheral roll

## Examples III to V

In these examples the same procedure as described in Example II was followed, except that the fibres were treated with aqueous solutions of potassium permanganate of different concentrations. All other aspects of the beating process, handsheet formation and tests were as described in Example II. The physical properties of the handsheets and the concentration of the respective aqueous solutions are set out in Table 3 below.

TABLE 3

| Example | Potassium permanganate concentration percent | Tear Strength (grams) | Burst Strength (p.s.i.) | Thickness (mils) | Tensile Strength (lbs./in.) | Shrinkage (percent) |
|---------|----------------------------------------------|-----------------------|-------------------------|------------------|-----------------------------|---------------------|
| III     | 1                                            | 46.4                  | 35.7                    | 6.3              | 16.3                        | 12.1                |
| IV      | 2.5                                          | 46.6                  | 17.2                    | 8.9              | 12.4                        | 12.4                |
| V       | 5                                            | 95.2                  | 25.7                    | 7.9              | 40.3                        | 11.6                |

speed for a period of 45 minutes. Handsheets were made by the conventional method using the British Standard sheet-making apparatus from which the chromium-plated surfacing plates had been removed on account of sticking. After being pressed, the handsheets were dried by an electric iron set, by a pyrometer, to a temperature of 107° C.  $\pm 2$ ° C. The sheets were again damped and re-dried to ensure complete flatness and stability. Physical strengths of the handsheets were tested on an Elmendorf tearing tester, a Mullen bursting strength tester, thickness by caliper, tensile strength by a Van der Korput tensile tester and shrinkage percent. The physical properties of the handsheets are set out in Table 1 below, all the results of the tests being corrected to standard substance 70 g.s.m.

TABLE 1

|                             |      |
|-----------------------------|------|
| Tear strength (grams)       | 14.3 |
| Burst strength (p.s.i.)     | 2.0  |
| Thickness (mils)            | 10   |
| Tensile strength (lbs./in.) | 1.6  |
| Shrinkage percent           | 15.6 |

TABLE 4

| Example | Tear Strength (grams) | Burst Strength (p.s.i.) | Thickness (mils) | Tensile Strength (lbs./in.) | Shrinkage (percent) |
|---------|-----------------------|-------------------------|------------------|-----------------------------|---------------------|
| VI      | 75.6                  | 17.2                    | 7.5              | 10.4                        | 14.5                |
| VII     | 91.8                  | 22.7                    | 7.9              | 14.4                        | 17.25               |

## Example II

100 grams dry weight undried acrylonitrile polymer fibres of 3 denier sold under the registered trademark Acrilan 1656 were cut into 1 inch staple lengths and rapidly stirred in 1.5 litres of a 2 percent aqueous solution of potassium permanganate maintained at a temperature of 100° C. on an electric hot-plate. After a period of five minutes the solution was decanted and the fibres were washed free of potassium permanganate in water at a temperature of 50°-60° C. The fibres were then spin-dried in a nylon net bag, thereafter air-dried and placed in a Clough laboratory beater. The beating and sheet-forming steps were identical to those described in Example I and the test carried out on the resulting handsheets were the same as those described in Example I. The physical properties of the handsheets produced are set out in Table 2 below.

TABLE 2

|                             |      |
|-----------------------------|------|
| Tear strength (grams)       | 21.2 |
| Burst strength (p.s.i.)     | 20.9 |
| Thickness (mils)            | 6.9  |
| Tensile strength (lbs./in.) | 30.1 |
| Shrinkage percent           | 14.2 |

## Example VIII

In this example 100 grams dry weight undried acrylonitrile polymer fibres of 3 denier and of the same composition as those employed in carrying out the preceding examples, but which had been stretched to the extent of 29 percent greater than those fibres and referred to as type "I" were cut to 1 inch staple lengths and subjected to precisely the same treatment and tests as in Example I. The physical properties of the handsheets produced are set out in Table 5 below.

TABLE 5

|                             |      |
|-----------------------------|------|
| Tear strength (grams)       | 89.4 |
| Burst strength (p.s.i.)     | 10.6 |
| Thickness (mils)            | 9.8  |
| Tensile strength (lbs./in.) | 17   |
| Shrinkage percent           | 17   |

## Example IX

In this example the same quantity of the "I" type fibres used in Example VIII were treated with a 2 percent aqueous solution of potassium permanganate maintained at a temperature of 100° C. for a period of five minutes and thereafter subjected to the beating and sheet-forming steps described in Example I, except that after a period of 15

minutes beating was discontinued as it was found that the fibres were fully split into sub-deniers. The physical properties of the handsheets are set out in Table 6 below.

TABLE 6

|                             |      |
|-----------------------------|------|
| Tear strength (grams)       | 94   |
| Burst strength (p.s.i.)     | 17.0 |
| Thickness (mils)            | 7.8  |
| Tensile strength (lbs./in.) | 28.3 |
| Shrinkage percent           | 18   |

10

## Example X to XII

In these examples the same procedure as described in Example II was followed, except that the fibres were treated with aqueous solutions of sodium hypochlorite of different concentrations. All other aspects of the beating process, handsheet formation and tests were as described in Example II. The physical properties of the handsheets and the concentration of the respective aqueous solutions are set out in Table 7 below.

TABLE 7

| Example | Sodium hypochlorite concentration (percent) | Tear Strength (grams) | Burst Strength (p.s.i.) | Thickness (mils) | Tensile Strength (lbs./in.) | Shrinkage (percent) |
|---------|---------------------------------------------|-----------------------|-------------------------|------------------|-----------------------------|---------------------|
| X       | 0.5                                         | 87.6                  | 12.2                    | 8.3              | 8.2                         | 12.1                |
| XI      | 1.0                                         | 84.5                  | 7.5                     | 8.3              | 9.8                         | 10.7                |
| XII     | 1.5                                         | 74                    | 7.9                     | 8.4              | 9.5                         | 10.6                |

## Example XIII

In this example the same procedure as described in Example II was followed, except that the fibres were treated for a period of 15 minutes in 1.5 litres of a 1.5 percent aqueous solution of sodium hypochlorite maintained at a temperature of 80° C. followed by soaking for a period of 15 minutes at a temperature of 20° C. in a 5 percent aqueous solution of sodium sulphite. All other aspects of the beating process, handsheet formation and tests were as described in Example II. The physical properties of the handsheets are set out in Table 8 below.

TABLE 8

|                             |       |
|-----------------------------|-------|
| Tear strength (grams)       | 35.5  |
| Burst strength (p.s.i.)     | 5.9   |
| Thickness (mils)            | 7.3   |
| Tensile strength (lbs./in.) | 5.7   |
| Shrinkage percent           | 10.75 |

## Examples XIV to XVI

In these examples the same procedure as described in Example II was followed, except that the fibres were treated for a period of 5 minutes at a temperature of 100° C. in 1.5 litres of aqueous solutions of ammonium persulphate of different concentrations. All other aspects of the beating process, handsheet formation and tests were as described in Example II. The physical properties of the handsheets and the concentration of the respective aqueous solutions are set out in Table 9 below.

TABLE 9

| Example | Ammonium persulphate concentration (percent) | Tear Strength (grams) | Burst Strength (p.s.i.) | Thickness (mils) | Tensile Strength (lbs./in.) | Shrinkage (percent) |
|---------|----------------------------------------------|-----------------------|-------------------------|------------------|-----------------------------|---------------------|
| XIV     | 2                                            | 45.2                  | 8.0                     | 8.1              | 5.5                         | 10                  |
| XV      | 5                                            | 53.0                  | 8.6                     | 7.9              | 5.6                         | 10                  |
| XVI     | 8                                            | 83.6                  | 20.0                    | 7.3              | 18.1                        | 10                  |

## Example XVII

In this example the same procedure as described in Example II was followed, except that the fibres were treated for a period of 5 minutes at a temperature of 100° C. in 5 litres of a 2 percent aqueous solution of potassium bichromate. All other aspects of the beating process, handsheet formation and tests were as described in Example II. The physical properties of the handsheets are set out in Table 10 below.

TABLE 10

|                             |      |
|-----------------------------|------|
| Tear strength (grams)       | 30.2 |
| Burst strength (p.s.i.)     | 4.9  |
| Thickness (mils)            | 8.0  |
| Tensile strength (lbs./in.) | 5.0  |
| Shrinkage percent           | 9.0  |

## Example XVIII

In this example the same procedure as described in Example II was followed, except that the fibres were treated for a period of 5 minutes at a temperature of 15 100° C. in 5 litres of a 2 percent aqueous solution of sodium perborate. All other aspects of the beating process, handsheet formation and tests were as described in Example II. The physical properties of the handsheets are set out in Table 11 below.

TABLE 11

|                             |      |
|-----------------------------|------|
| Tear strength (grams)       | 35.0 |
| Burst strength (p.s.i.)     | 7.5  |
| Thickness (mils)            | 7.9  |
| Tensile strength (lbs./in.) | 5.0  |
| Shrinkage percent           | 9.0  |

## Example XIX

In this example the same procedure as described in Example II was followed, except that the fibres were treated for a period of 15 minutes at a temperature of 100° C. in 5 litres of a 2 percent aqueous solution of potassium persulphate. All other aspects of the beating process, handsheet formation and tests were as described in Example II. The physical properties of the handsheets are set out in Table 12 below.

TABLE 12

|                  |          |      |
|------------------|----------|------|
| Tear strength    | grams    | 11.5 |
| Burst strength   | p.s.i.   | 12.3 |
| Thickness        | mils     | 7.9  |
| Tensile strength | lbs./in. | 11.8 |
| Shrinkage        | percent  | 10.5 |

55 From the above tables it will be seen that the physical properties of the handsheets prepared from fibers which had undergone treatment with an oxygen-forming agent

in accordance with the invention as described in Examples II to VII and IX to XIX were superior to the physical properties of the handsheets prepared in accordance with Examples I and VIII where the fibers were not subjected to treatment with an oxygen-forming agent.

It will be understood that although the foregoing examples describe some of the more specific details of the invention, they are given merely for the purposes of illustration and the invention is not limited thereto. Thus, although in the examples the invention has been described

in connection with the preparation of handsheets, it is applicable to the continuous production of paper sheets or webs of indefinite lengths by conventional means.

The concentration of the aqueous solution of the oxygen-forming agent can be varied to suit particular requirements and may range from  $\frac{1}{2}$  percent to 10 percent. Similarly, the temperature of the solution can vary from 10° C. to 100° C. and the time during which the fibres undergo treatment by the solution can be varied as may be found necessary.

We claim:

1. A process for the treatment of fibres formed from an acrylonitrile polymer containing at least 80 percent by weight of acrylonitrile to render said fibres suitable for use in the manufacture of paper comprising the steps of reducing said fibres to staple lengths, immersing said fibres in an aqueous solution consisting essentially of from about .5 percent to 10 percent of an oxygen-forming agent wherein said agent is a member selected from the group consisting essentially of potassium permanganate, sodium hypochlorite, ammonium persulphate, potassium bichromate, sodium perborate and potassium persulphate at a temperature in the range of from 10° C. to 100° C. for 5 to 30 minutes thereby to partially disrupt said fibres, washing said fibres to remove said oxygen-forming agent and drying said fibres.

2. A process for the manufacture of paper from fibres produced from an acrylonitrile polymer containing at least 80 percent by weight of acrylonitrile comprising the steps of reducing said fibres to staple lengths, immersing said fibres in an aqueous solution composed essentially of from about .5 to 10 percent of an oxygen-forming agent wherein said agent is a member selected from the group consisting of potassium permanganate, sodium hypochlorite, ammonium persulphate, potassium bichromate, sodium perborate and potassium persulphate at a temperature in the range of from 10° C. to 100° C. for 5 to 30 minutes thereby to partially disrupt the fibres, washing said fibres to remove said oxygen-forming agent, drying said fibres, beating said fibres in an aqueous dispersion and forming said fibres into a web.

3. A process according to claim 1, wherein said polymer is a blend of a copolymer of 80 to 99 percent by weight of acrylonitrile and 1 to 20 percent by weight of vinyl acetate and a copolymer of 10 to 70 percent by weight of acrylonitrile and 30 to 90 percent by weight of a vinyl-substituted tertiary heterocyclic amine, said blend having an overall vinyl-substituted tertiary heterocyclic amine content of from 2 to 10 percent based on the weight of the blend.
4. A process according to claim 1 wherein said fibres consist of a copolymer of at least 80 percent by weight of acrylonitrile and up to 20 percent by weight of another copolymerizable mono-olefinic monomer.
5. A process for the treatment of fibres formed from an acrylonitrile polymer containing at least 80 percent by weight of acrylonitrile according to claim 1.
6. A process for the manufacture of paper from fibres produced from an acrylonitrile polymer containing at least 80 percent of acrylonitrile according to claim 2.
7. Fibres containing at least 80 percent by weight of acrylonitrile when treated by the process in accordance with claim 1.
8. Paper when produced by the process in accordance with claim 2.
9. A process according to claim 2 wherein said fibres consist of a copolymer of at least 80 percent by weight of acrylonitrile and up to 20 percent by weight of another copolymerizable mono-olefinic monomer.

#### References Cited

##### UNITED STATES PATENTS

|           |        |       |       |         |
|-----------|--------|-------|-------|---------|
| 3,127,233 | 3/1964 | Lowes | ----- | 8—111   |
| 3,232,824 | 2/1966 | Bader | ----- | 162—157 |

HOWARD R. CAINE, *Primary Examiner.*

U.S. Cl. X.R.

40 8—111